

April 15, 1930.

R. J. POMEROY

1,755,129

METHOD OF MAKING COMPOSITE PHOTOGRAPHS

Filed July 14, 1926

Fig. 1



LATENT IMAGE OF ACTION

Fig. 2



DEVELOPED - BLACK  
AND WHITE NEGATIVE

Fig. 3



BLEACHED  
(RED-BROWN)

Fig. 4



INTENSIFIED  
(BROWN-BLACK)

Fig. 5



REDEVELOPED

Fig. 6



EXPOSED TO  
BACKGROUND SCENE

Fig. 7



DEVELOPED

Fig. 8



COMPOSITE NEGATIVE  
AFTER FIXING

Fig. 9



LATENT IMAGE OF ACTION

Fig. 10



DEVELOPED - BLACK  
AND WHITE NEGATIVE

Fig. 11



COATED WITH  
PIGMENTED CASEIN

Fig. 12



BLEACHED - CASEIN  
HARDENED OVER IMAGE

Fig. 13



WASHED - CASEIN REMOVED  
EXCEPT OVER IMAGE

Fig. 14



EXPOSED TO BACKGROUND SCENE

Fig. 15



DEVELOPED AND FIXED

Fig. 16



COMPOSITE NEG AFTER REMOVAL  
OF CASEIN FROM ACTION IMAGE

Inventor

Roy J. Pomeroy.

  
Attorney.

## UNITED STATES PATENT OFFICE

ROY J. POMEROY, OF LOS ANGELES, CALIFORNIA, ASSIGNOR OF ONE-HALF TO  
FAMOUS PLAYERS-LASKY CORPORATION, OF LOS ANGELES, CALIFORNIA, A COR-  
PORATION OF NEW YORK

## METHOD OF MAKING COMPOSITE PHOTOGRAPHS

Application filed July 14, 1926. Serial No. 122,502.

This invention has to do with methods of making composite photographs, or with what is more commonly known as a method of double exposure; the general object of such a method being to obtain upon a single photograph or film two or more images taken at different times or places. In motion picture photography such double exposure methods are used for the purpose of apparently placing an action in a scene or before a background foreign to the actual action.

In most, if not all, the present schemes of double exposure, a plurality of films must be used, it being a more or less common practice to take the action on one film and the background on another film, then print the two original films onto another on which the composite is obtained. It is one of the objects of this invention to provide a method of obtaining composite photographs or double exposure effects with the use of only one film or negative; and the invention also has further objects in the direction of simplicity, accuracy, ease of manipulation, etc., all as will best be understood from a consideration of the following detailed specification. In this specification I set out the general method which is the subject matter of this application and which typifies and illustrates the invention, and also set out various modifications as to procedure and as to substances which may be used in the method. Certain specific modifications are included in the broad subject matter here, but are the specific subject matter of a companion application filed on even date herewith, Serial Number 122,503.

I shall explain the method as for making a composite picture to show an action in a scene or before a background not actually associated with the action; but it will be well understood that the method can be used for obtaining composite photographs of any desired subject.

Reference is had throughout the specification to the accompanying drawings, in which:

Fig. 1 shows the negative after exposure to the action;

Fig. 2 shows the exposed negative after developing;

Fig. 3 shows the negative after bleaching; Fig. 4 shows the bleached negative intensified;

Fig. 5 shows the intensified negative after redeveloping;

Fig. 6 shows the negative after exposure to the background scene;

Fig. 7 shows the negative after developing;

Fig. 8 shows the composite negative resulting after bathing in fixing solution;

Fig. 9 shows another negative after exposure to action;

Fig. 10 shows the exposed negative after developing;

Fig. 11 shows the negative after being coated with pigmented casein;

Fig. 12 shows the negative after bleaching;

Fig. 13 shows the negative with the casein washed away except the hardened portion over the action image;

Fig. 14 shows the negative after exposure to the background scene;

Fig. 15 shows the negative after developing and fixing; and

Fig. 16 shows the composite negative resulting after removal of the hardened casein from the action image.

The negative is first exposed to the action against a black or non-actinic ground so that the exposed negative will then carry a latent image 10 of the action in a ground unaffected by light (see Fig. 1).

Next this film is developed in the usual manner but is not fixed at this time. The film then shows the image 11 of the action in a clear ground; but the clear ground and the unreduced silver salts in the image area are still actinic. See Fig. 2, wherein shading of image does not represent color but black and white tones.

Next, the film is bleached with a water solution of quinones, potassium bromide and acetic acid. A solution suitable for this purpose will contain by weight: water 96.65 percent; quinones .55 percent; potassium bromide 2.8 percent. A slight amount of acetic acid may be used. This bleach has no effect on the unexposed and undeveloped portions of the film, but transforms the developed parts of the film to a reddish brown color, the

metallic silver being probably transformed to silver oxy-bromide. See Fig. 5, where the shading represents color.

Then the image on the film is intensified by 5 treating the film with a water solution of potassium or sodium carbonate or hydroxide. This solution again has no effect on the unexposed portions but intensifies the image to a deep brown black (see Fig. 4). Next the film 10 is re-developed with any non-staining developer, such as amidol (diamidophenol hydrochloride) or glycine (para-oxy-phenylglycine). Such developers will again metallize the silver but will not stain the film 15 (see Fig. 5).

Instead of intensifying, after bleaching the film may be treated with a desensitizer that will act selectively on the bleached area. For instance, pheno-safranine, sodium bichromate, or pina-kryptol green, may be used for 20 that purpose. These desensitizers appear to owe their selective action upon the film to the prior bleaching treatment.

Next the film with its redeveloped image is 25 washed and dried, ready for the second exposure. At this stage of the procedure the film has in it a redeveloped image. The original exposure has preferably been a slight over-exposure; and the intensification 30 of the image after bleaching is sufficient when the film is re-exposed to hold back further light action throughout the area of the first images. It will be understood that the intensification products are still present in the 35 film at this stage of the procedure, surrounding the redevelopment products. The initial bleaching has transformed the developed metallic silver to a silver compound and is then intensified or "spread" by the intensification 40 treatment.

With the film in this condition, the second exposure is then made, such exposure being typically to a scene or background. As will now be understood, this second exposure does 45 not affect the previously exposed portions, but only the previously unexposed portions. The negative now carries a latent image 12 of the background scene (see Fig. 6).

Finally the film is again developed and 50 then finally fixed (Figs. 7 and 8). In this second development a developer is used as before, the developer having no effect on the intensification products, but bringing out the background image 13. A suitable fixer for 55 use in the process is hypo. The fixing operation not only removes the unexposed silver salts, but also removes all the intensification product to the point where the first image appears normal, thus leaving only the two 60 normal images.

In case a desensitizer is used instead of intensifying, the subsequent steps of the process are the same, the desensitizer being removed in the hypo.

65 The intensification products obtained in

this method are a good mordant for certain basic dyes, and the action image can be dyed before the second exposure so that the action image will show up in color in the final film. And this, as will readily be understood, can 70 be done without affecting parts of the film where no intensification products are present. Although various basic dyes may be used to obtain different colors, I may mention typically the following: fuchsine, safranine 75 or chrysoidin.

In a variation of the method as here described, the film is first exposed to the action before the black ground and is then developed, as before described (Figs. 9 and 10). Then next the film is coated with a thin layer 80 of casein or other colloid carrying an opaque or non-actinic pigment which is neutral to the chemicals used in the method. The pigment known as Indian red is suitable for this 85 purpose (see Fig. 11).

Then the coated film is next bleached with a solution capable of hardening the gelatine and the casein where there is present metallic silver. A quinone bleach, such as described before or a copper bromide bleach, is suitable for this purpose, but any bleach that will harden the casein locally may be used. Such a bleach transforms the silver and 90 hardens the gelatine and the casein by action with the chemical by-products of the silver bleaching. This hardened casein carrying its opaque or non-actinic pigment then becomes the protector of the previously exposed 95 portions during the next exposure; and thus performs generally the function that is performed in the first described method by the intensification product. The film then appears as in Fig. 12.

Next the film is treated with dilute alkaline 105 solution such as sodium or potassium hydroxide solution which washes off the unaffected or unhardened parts of the casein; so that the previously unexposed portions of the film are then uncovered, while the previously exposed portions are left covered with the pigmented casein (see Fig. 13).

Then the film is washed and dried as before, and re-exposed as before (Fig. 14); and then 115 is finally developed with any suitable developer as amidol or glycine (see Fig. 15). This final development not only re-develops the bleached silver of the first image, but also develops the image of the second exposure if not previously developed. The first image 120 may be redeveloped before the second exposure in the same manner as in the other method.

Then the film is finally fixed with any suitable fixing solution as hypo; the pigmented casein is finally removed from the initial image by a stronger wash in alkaline solution (see Fig. 16).

With proper control of the several operations involved in the methods herein de- 130

scribed, the two final images are made to match each other very accurately, so that the action image then appears as if it were naturally in the background image. Proper control for these purposes is not difficult, being concerned mainly with the obtainance of the correct image intensities and the correct amount of bleaching and spread of the intensification products or of the hardening of the casein, so that the intensification products or the casein will correspond as closely as possible with the outlines of the original action image.

I claim:

- 15 1. The herein described method of producing composite photographs, that includes first exposing a limited portion of a fresh actinic surface to obtain thereon a first image, developing said first image, bleaching and intensifying the developed image, redeveloping said image, exposing other portions of the surface, developing the whole surface with a developer that will not further develop the products of intensification, and finally fixing.
- 25 2. The herein described method of producing composite photographs, that includes first exposing a limited portion of a fresh actinic surface to obtain thereon a first image, developing said first image, the first exposure being over normal to obtain a dense image, bleaching the developed image with a quinone bleach to transform the reduced silver, intensifying the bleached image with an alkali hydrate to obtain intensification products immune to further light action, redeveloping the image and carrying such redevelopment to the point of obtaining the normal image, leaving the remainder of the intensification products unaffected, exposing other portions of
- 30 the surface, developing the whole surface, and finally fixing with a fixing solution that removes the intensification products as well as the undeveloped actinic silver salts.

In witness that I claim the foregoing I have hereunto subscribed my name this 30th day of June 1926.

ROY J. POMEROY.